

# United States Patent Office

2,874,120

Patented Feb. 17, 1959

1

2,874,120

## LUBRICATING OIL COMPOSITIONS

Forrest J. Watson and Rupert C. Morris, Berkeley, and John L. Van Winkle, San Lorenzo, Calif., assignors to Shell Development Company, New York, N. Y., a corporation of Delaware

No Drawing. Application August 17, 1956  
Serial No. 604,618

7 Claims. (Cl. 252—32.5)

This invention relates to lubricants, and particularly to lubricating compositions which are suitable for use in equipment operating under extreme conditions, such as under extreme pressure, variable speed and wide temperature conditions.

It has been observed that certain types of phosphorus acids as defined more specifically hereinafter, impart outstanding extreme pressure properties to various lubricating compositions. However, these very effective agents are in general undesirable because they promote wear and cause corrosion.

The phosphorus acids referred to can be represented by the general formula:



wherein R is a polyhalohydrocarbyl radical and preferably a perchloroalkyl radical.

The art discloses that some of the undesirable properties of these acids can be overcome by forming secondary amine salts of these polyhalohydrocarbyl phosphonic acids such as the di(2-ethyl-hexyl)amine salts of butyl trichloromethylphosphonic acid. However, in many cases these amine salts lack desired oil solubility and in storage tend to precipitate from the oil and form sludge.

It has now been discovered that certain amine salts of monochloroalkyl phosphonic acids, the acid being represented by the formula:



wherein R is a monochloroalkyl radical of from 1 to 4 and preferably 1 to 2 carbon atoms and the chlorine atom is in the alpha position relative to the phosphorus atom, possess outstanding extreme pressure and load carrying properties, have good oil solubility and are non-corrosive and non-staining when in contact with ferrous or non-ferrous metals.

2

chloroalkyl phosphonic acids are highly branched aliphatic primary amines or aliphatic secondary amines of at least 8 carbon atoms. Of the highly branched aliphatic primary amines, the tertiary alkyl primary amines

5 are preferred and they can be prepared by any suitable means such as described in the U. S. Office of the Publication Board Report No. 88843. Other highly branched primary amines can be prepared by converting primary branched chain olefins as fully described by P. W. Sher-

10 wood in the Oil and Gas Journal, June 9, 1949, page 71, and in the February 1953 issue of Petroleum Processing, to the corresponding nitriles and converting the nitrile to the amine by catalytic hydrogenation. Another method is to convert highly branched alcohols to the corresponding halides and to form the amines derived from the halide in the customary manner such as by reacting with ammonia.

It has been found that the tertiary alkyl primary amines, containing as the tertiary alkyl radical, the radical of poly-

20 isobutylene, polypropylene and mixtures thereof are particularly effective for the present purpose and they constitute a preferred class of amines for the practice of the invention. Accordingly, 1,1,3,3-tetramethylbutylamine

25 (from the amination of diisobutylene), 1,1,3,3,5,5-hexamethylhexylamine (from triisobutylene), 1,1,3,3,5,5,7,7-

octamethyloctylamine (from tetraisobutylene) and 1,1,3,3,5,5,7,7-

30 9,9-decamethyldecylamine (from penta-isobutylene) are specific preferred amines, which are suitably used individually or as mixtures thereof. In addition to these tertiary alkyl primary amines, tertiaryalkylmethyl

2,4,4,6,6-hexamethylheptylamine and the like are suitable.

Other tertiary alkyl primary amines which can be used include the C<sub>8</sub> and higher amines of this type mentioned in U. S. Patents 2,160,058, 2,606,923 and 2,611,782, such as tert-tridecylamine



as well as isoheptyldiethylcarbinylamine, isoocetylethylpropylcarbinylamine, and the like. Primary amines of this type are commercially available from Rohm and Haas Company under the trade name of "Primenes," specific products being "Primene 81-R," which is a mixture of primary alkylamines containing from about 12 to 15 carbon atoms and "Primene JM-T," which is a similar tertiary alkylamine mixture containing an average of about 18 to 24 carbon atoms.

The following are the properties of some amines which can be used to form the amine salts for use in lubricating compositions of this invention.

Table I.—Properties

|                               | Tertiary-octylamine                                    | Alkylamine 81-R<br>A <sub>1</sub>                                                                                                                   | Alkylamine JM-T<br>A <sub>3</sub>                                                                                                                   |
|-------------------------------|--------------------------------------------------------|-----------------------------------------------------------------------------------------------------------------------------------------------------|-----------------------------------------------------------------------------------------------------------------------------------------------------|
| Formula.....                  | t-C <sub>8</sub> H <sub>17</sub> NH <sub>2</sub> ..... | Principally t-C <sub>12</sub> H <sub>25</sub> NH <sub>2</sub> to<br>t-C <sub>15</sub> H <sub>31</sub> NH <sub>2</sub> .<br>Principally 185-227..... | Principally t-C <sub>18</sub> H <sub>37</sub> NH <sub>2</sub> to<br>t-C <sub>21</sub> H <sub>49</sub> NH <sub>2</sub> .<br>Principally 269-353..... |
| Molecular weight.....         | 128.....                                               | 191.....                                                                                                                                            | 315.....                                                                                                                                            |
| Average molecular weight..... | 131.....                                               | 0.812.....                                                                                                                                          | 0.840.....                                                                                                                                          |
| Specific gravity, 25° C.....  | 0.771.....                                             | 1.423.....                                                                                                                                          | 1.456.....                                                                                                                                          |
| Refractive index, 25° C.....  | 1.423.....                                             | 5-90% at 223-240° C. (760 mm.)                                                                                                                      | 5-70% at 265-308° C. (760 mm.)                                                                                                                      |
| Boiling point (or range)..... | 137-143° C. (760 mm.)                                  |                                                                                                                                                     |                                                                                                                                                     |

The acid portion used to make either the partial or full amine salt can be prepared by the method described by Barnard et al. in the Canadian Journal of Chemistry, vol. 31, 1953, pages 976 to 983. Acids of this type include monochloromethyl-, monochloroethyl-, monochloropropyl-, monochloroisopropyl-, monochlorobutyl- and monochloroisobutylphosphonic acids, in which the chlorine is in the alpha position.

The amines which form effective salts of the mono-

65 fective salts of the phosphorus acids are preferably those aliphatic and cycloaliphatic amines which contain from 10 to 36 carbon atoms. Illustrative of such amines are diethylamine, dihexylamine, di(2-ethylhexyl) amine, dioctylamine, didecylamine, diodecylamine, ditetradecylamine, dihexadecylamine, dioctadecylamine, dibromodioctadecylamine, isopropylolylamine, diricinoleylamine, butyricinoleylamine, butyl-2-ethylhexylamine, dilauryl-

amine, methyloleylamine, ethyloctylamine, isoamylhexylamine, dicyclohexylamine, dicyclopentylamine, cyclohexyloctylamine, cyclohexylbenzylamine, benzyloctylamine, benzyl-2-ethylhexylamine, dodecyl-2-ethylhexylamine, (1-isobutyl-3-methylbutyl)-3,3,5-methylcyclohexylamine, di-(1-isobutyl-3-methylbutyl)amine; N-n-dodecylidethylenetriamine, N-n-tetradecylidethylenetriamine, octylethylene diamine N-2-ethylhexyl N-hexadecyl triethylene tetraamine, heptyl trimethylene diamine, N-tetradecyl tripropylene tetramine, 3-hexyl-morpholine, and the like.

The mono- and diamine salts can be represented by the formulas:



and



wherein R is the same as defined in Formula II, and A is a long-chain highly branched aliphatic primary amine or aliphatic secondary amine, having at least 8 carbon atoms and higher such as up to 30 carbon atoms in the molecule.

The amine salts of the monochloroalkyl phosphonic acids and mixtures thereof as described can be prepared by interacting the selected amine with monochloroalkylphosphonic acid in a suitable solvent if desired and under suitable conditions such as mixing at elevated temperature, stirring and heating. Salts produced in the foregoing or equivalent manner can be purified by recrystallization from suitable solvents or other means which will be apparent to those skilled in the art. For example, monochloromethylphosphonic acid was reacted at a temperature of around 100° C. with a mixture of t-C<sub>18</sub>H<sub>37</sub>NH<sub>2</sub> to t-C<sub>24</sub>H<sub>49</sub>NH<sub>2</sub> (A<sub>3</sub>) in an amount sufficient to neutralize the total acidity of the acid, namely, one mole of the acid for two moles of the amine. The product is represented by the formula



or equivalently



This salt was completely soluble in mineral oil, was non-corrosive and possessed excellent extreme pressure properties. Using two moles of a mixture of t-C<sub>12</sub>H<sub>25</sub>NH<sub>2</sub> to t-C<sub>15</sub>H<sub>35</sub>NH<sub>2</sub> (A<sub>1</sub>) in forming the salt, the final product had the formula



or equivalently



Another excellent non-corrosive extreme pressure additive having good oil solubility was prepared by using only half the stoichiometric amount of amine (A<sub>3</sub>) required to neutralize the total acidity of monochloromethanephosphonic acid. The product had the formula



or equivalently



The partially neutralized highly-branched-chain primary amine salts which are specifically preferred include: t-C<sub>12</sub>H<sub>25</sub>NH<sub>2</sub>, t-C<sub>12</sub>H<sub>25</sub>NH<sub>2</sub> to t-C<sub>15</sub>H<sub>31</sub>NH, t-C<sub>18</sub>H<sub>31</sub>NH<sub>2</sub> to t-C<sub>24</sub>H<sub>49</sub>NH<sub>2</sub>, dimethylenopentylcarbinyl amine, tert. tridecyl amine salts of monochloromethyl phosphonic acid, mono-alpha-chloroethylphosphonic acid.

The secondary amine salts which are specifically preferred include: di-2-ethylhexylamine, di-1-isobutyl-3-methylbutylamine, didecylamine, dioctadecylamine, isopropylolylamine, butyl-2-ethylhexylamine, dicyclohexylamine salts of monochloromethylphosphonic acid mono-alpha-chloroethylphosphonic acid.

The amine salts of the monochloroalkylphosphonic acids can be used in amounts ranging from about 0.01% to about 10% and preferably between 0.1% and 5% by weight.

Base oils to which agents of this invention are added may be selected from a variety of natural oils such as paraffinic, naphthenic and mixed base mineral oils having a viscosity range such as from 50 SUS at 100° F., up to 250 SUS at 210° F. In addition, synthetic oils

may be used such as polymerized olefins, alkylated aromatics, polyalkyl silicone polymers, e. g., liquid dimethyl silicone polymer, other silicone polymers, H<sub>2</sub>S-adducts of unsaturated ethers and thioethers, e. g. H<sub>2</sub>S adduct of dialkyl ether, esters, e. g., di(2-ethylhexyl)sebacate. Mixtures of natural and synthetic oils can be used.

The outstanding properties which compositions of this invention possess is evidenced from the data presented in Table II. The L-13 rust test is described in the 1946 CRC Handbook published by the Co-ordination Research Council; the four-ball test is described in Engineering, vol. 136, July 13, 1933; the bearing stain test consists of immersing a small clean Timken bearing in the composition being tested and heating the composition to 150° C. for 65 hours. The bearing is removed, solvent washed and staining (10=bearing stain and 0=clean) observed in the cup and cone of the bearing. The reverse hypoid score load in H. P. is measured on the hypoid gear machine operated at 4000 R. P. M., giving results similar to the L-19 test described in the CRC Handbook mentioned above.

Table II  
45 MINERAL OIL BASE SAE 90, ADDITIVE PRESENT IN AMOUNT OF 0.12% P

|    | Additive                                                                        | L-13,<br>4 hrs.,<br>82° C. | Bearing<br>stain<br>test—<br>65 hrs.,<br>150° C.,<br>cup/cone;<br>10=bear-<br>ing stain,<br>0=clean | Reversed<br>hypoid<br>score<br>(L-19)—<br>load,<br>H. P. | 4-ball<br>ISL, kg. |
|----|---------------------------------------------------------------------------------|----------------------------|-----------------------------------------------------------------------------------------------------|----------------------------------------------------------|--------------------|
| 50 |                                                                                 |                            |                                                                                                     |                                                          |                    |
| 55 | Salt <sup>1</sup> of di-2-ethylhexylamine and monochloromethyl phosphonic acid. | Pass...                    | 4/4                                                                                                 | -----                                                    | 200-224            |
|    | Salt <sup>1</sup> of amine "A" of Table I and—                                  |                            |                                                                                                     |                                                          |                    |
|    | monochloromethyl phosphonic acid.                                               | ...do...                   | 2/1                                                                                                 | 154                                                      | 158-178            |
|    | Alpha-chloroethyl phosphonic acid.                                              | ...do...                   | -----                                                                                               | 140                                                      | 158-178            |
|    | Beta-chloroethyl phosphonic acid.                                               | Fail...                    | 8/8                                                                                                 | 70                                                       | 141-158            |
|    | None.....                                                                       | ...do...                   | -----                                                                                               | -----                                                    | 40-45              |

65 SULFURIZED PALE OIL BASE ADDITIVE PRESENT IN AMOUNT OF 0.12% P

|                                                                                 |       |       |       |         |
|---------------------------------------------------------------------------------|-------|-------|-------|---------|
| Salt <sup>2</sup> of amine "A" of Table I and monochloromethyl phosphonic acid. | ----- | ----- | ----- | 224-251 |
|---------------------------------------------------------------------------------|-------|-------|-------|---------|

70 PALE OIL BASE 170 SUS AT 100° F., PRESENT IN AMOUNT OF 0.12% P

|                                                                                 |       |       |       |         |
|---------------------------------------------------------------------------------|-------|-------|-------|---------|
| Salt <sup>2</sup> of amine "A" of Table I and monochloromethyl phosphonic acid. | ----- | ----- | ----- | 224-250 |
|---------------------------------------------------------------------------------|-------|-------|-------|---------|

UCON D6B-190B<sup>3</sup> BASE ADDITIVE PRESENT IN AMOUNT OF 0.12% P

|                                                                                     |  |  |         |   |
|-------------------------------------------------------------------------------------|--|--|---------|---|
| Salt <sup>2</sup> of amine "A" of Table I and—<br>monochloromethyl phosphoric acid. |  |  | 178-200 | 5 |
| None.                                                                               |  |  | 56- 63  |   |

## DI-2-ETHYL HEXYL SEBACATE BASE ADDITIVE PRESENT IN AN AMOUNT OF 0.12% P

|                                                                                     |  |  |         |    |
|-------------------------------------------------------------------------------------|--|--|---------|----|
| Salt <sup>1</sup> of amine "A" of Table I and—<br>monochloromethyl phosphoric acid. |  |  | 200-224 | 10 |
| None.                                                                               |  |  | 40- 45  |    |

<sup>1</sup> Total acid neutralized.<sup>2</sup> Strong acidity neutralized only.<sup>3</sup> Dibutyl derivative of polyoxypropylene glycol having a viscosity of 190 SUS at 100° F.

In addition to the additives already described, lubricating oil compositions contemplated herein may contain other agents, such as pour-point depressants, oiliness agents, blooming agents, compounds for enhancing the viscosity index of the lubricating oil, peptizing agents, metal deactivators, etc.

We claim as our invention:

1. A lubricating oil composition comprising a major amount of a mineral lubricating oil and from about 0.01% to about 10% by weight of an oil-soluble aliphatic amine salt of a monochloroalkylphosphonic acid containing from 1 to 4 carbon atoms in the alkyl group and wherein the chlorine atom is on the alpha carbon to the phosphorus atom, the amine portion of the salt being a branched-chain-aliphatic amine having from 8 to 24 carbon atoms and selected from the group consisting of primary and secondary amines.

2. A lubricating oil composition comprising a major amount of mineral lubricating oil and from about 0.01% to about 10% by weight of an oil soluble branched-chain-C<sub>8-24</sub>-aliphatic primary amine salt of monochloro C<sub>1-4</sub> alkyl phosphonic acid wherein the chlorine is on the alpha carbon to the phosphorus atom.

3. A lubricating oil composition comprising a major amount of mineral lubricating oil and from about 0.01% to about 10% by weight of an oil soluble branched-chain-C<sub>8-24</sub>-aliphatic secondary amine salt of monochloro C<sub>1-4</sub> alkyl phosphonic acid wherein the chlorine is on the alpha carbon to the phosphorus atom.

4. A lubricating oil composition comprising a major amount of mineral lubricating oil and from about 0.1 to about 5% by weight of di-2-ethylhexylamine salt of monochloromethylphosphonic acid.

5. A lubricating oil composition comprising a major amount of mineral lubricating oil and from about 0.1 to about 5% by weight of a mixture of t-C<sub>18</sub>H<sub>37</sub>NH<sub>2</sub> to t-C<sub>24</sub>H<sub>49</sub>NH<sub>2</sub> amine salt of monochloromethylphosphonic acid.

6. A lubricating oil composition comprising a major amount of mineral lubricating oil and from about 0.1 to about 5% by weight of a mixture of t-C<sub>12</sub>H<sub>25</sub>NH<sub>2</sub> to C<sub>15</sub>H<sub>31</sub>NH<sub>2</sub> amine salt of monochloromethylphosphonic acid.

7. A lubricating composition according to claim 1, wherein the monochloroalkylphosphonic acid is alpha-chloroethylphosphonic acid.

30

## References Cited in the file of this patent

## UNITED STATES PATENTS

|              |           |               |
|--------------|-----------|---------------|
| 2,169,185    | Shoemaker | Aug. 8, 1939  |
| 2,683,691    | Thorpe    | July 13, 1954 |
| 35 2,777,819 | Williams  | Jan. 15, 1957 |